

## UNITED STATES PATENT OFFICE.

HERBERT MEYER, OF BERLIN-TREPTOW, GERMANY, ASSIGNOR, BY MESNE ASSIGNMENTS, TO AGFA ANSCO CORPORATION, OF BINGHAMTON, NEW YORK, A CORPORATION OF NEW YORK.

COMBINED DESENSITIZER AND DEVELOPER AND PROCESS OF DESENSITIZING AND DEVELOPING.

No Drawing. Application filed September 8, 1927, Serial No. 218,365, and in Germany November 13, 1926.

The present invention relates to new photographic developers, more particularly to photographic developers comprising the cyanide of a heavy metal. It relates further 5 more to the process of developing photographic surfaces with the aid of the new developers.

I have found that the cyanides of the heavy metals act as good desensitizers when added 10 to a photographic developing agent i. e. their presence in the developing agent permits photographic surfaces to be developed either wholly or in greater part in full light without diminishing the latent image. As compared with the known desensitizing dyestuffs the cyanides of the heavy metals have the 15 advantage that they do not color the developer, or the developed sensitive materials. In addition they remain active for a much longer 20 time in concentrated developing solutions for example, in concentrated hydroquinone-developers.

I have furthermore found that the cyanides of the heavy metals have a pronounced anti-fog action so that with their aid not only the 25 known time developers are improved, but any developing agent can be made suitable for time development.

I prefer to use mercury cyanide which is 30 especially efficient, but the cyanides of the other heavy metals may be used also, as for instance cobalt- or cadmium-cyanide, although they are not quite as efficient as mercury cyanide.

Generally it will be sufficient to add about 35 0.03 parts by weight of mercury cyanide to the developing agent. It makes no difference as to the action of the cyanide whether it is added to the developing agent itself or to the solution formed therefrom.

*Example 1.*—To a monomethyl-para-aminophenol-sulphate-hydroquinone developer, mercuric cyanide is added in the proportion of 0.3 gram to 1000 cc. of the developer. The 40 exposed material to be developed is developed

in a room having usual dark room illumination for  $\frac{1}{2}$  to 2 minutes, whereupon a further development is carried out in a bright yellow light, as is usual in operating with the known dyestuff desensitizers. 50

*Example 2.*—A monomethyl-para-aminophenol-sulphate-hydroquinone developer, in which the exposed material to be developed would acquire a considerable fog as the effect of 10 minutes development, receives an 55 addition of 0.3 gram of mercuric cyanide per 1000 cc. of developer. The same material may now be developed under normal dark room illumination in this developer containing cyanide for 20-50 minutes without showing appreciable fog after fixing. 60

I claim:

1. As new compositions of matter photographic developers comprising the cyanide of a heavy metal. 65
2. As new compositions of matter photographic developers comprising mercury cyanide.
3. As a new composition of matter a photographic developer comprising mercury cyanide, monomethyl-para-aminophenol-sulphate and hydroquinone. 70
4. A process of desensitizing and developing exposed silver halide sensitized elements, which comprises subjecting them to the action of a photographic developer containing a cyanide of a heavy metal. 75
5. A process of desensitizing and developing exposed silver halide sensitized elements, which comprises subjecting them to the action of a photographic developer containing mercury cyanide. 80
6. A process of desensitizing and developing exposed silver halide sensitized elements, which comprises subjecting them to the action of a photographic developer containing mercury cyanide, monomethyl-para-aminophenol-sulphate and hydroquinone. 85

In testimony whereof, I affix my signature.

DR. HERBERT MEYER.